

## UNITED STATES PATENT OFFICE

2,537,001

DIAZOTYPE LAYERS HAVING CYAN ACETYL  
AMIDES AS AZO COMPONENTS

William H. von Glahn, Loudonville, and Lester N. Stanley, Delmar, N. Y., assignors to General Aniline & Film Corporation, New York, N. Y., a corporation of Delaware

No Drawing. Application August 6, 1947,  
Serial No. 766,875

6 Claims. (Cl. 95—6)

1

This invention relates to a diazotype process and more particularly to the use of organic esters and nitriles containing an active methylene group as the azo components in the light sensitive layer of a diazotype reproduction medium or in a developing solution for the exposed diazotype image.

In the reproduction of mechanical drawings, printed material, pictures or other originals to be copied, it is of particular advantage in many cases to make first an intermediate print or transition print on a transparent diazotype copying material by exposing the transparent sensitized diazotype material to actinic rays, such as ultraviolet light, by either the printing through or reflex process and then developing the diazotype material. The development of such diazotype prints may be carried out by any of the developing methods known to the art for development of exposed diazotype materials. Thus, where a two-component system is employed containing the azo component in the light sensitive layer with the diazo compound, development is effected by passing the exposed diazotype through ammonia vapors, and where a one-component system is employed which contains the diazo compound as the only dye component in the light sensitive layer, the image is developed by treating the exposed diazotype with an alkaline solution containing the azo component by a dipping or fog spraying method. The image thus produced on the transparent intermediate or transition diazotype print can be used for reproduction of further diazotype prints of high contrast. If desired, they can also be used for the reproduction of the image on any suitable photoprinting material such as silver halide photographic paper and Van Dyke prints and blueprints.

This method of producing transition diazotype prints is particularly useful when it is desired to make a number of reproductions from a frail or valuable original which would be adversely affected, if not destroyed, in the repeated exposures necessary to make the desired number of copies. It is essential in the so-called reflex process, where the diazotype copy material is superimposed on the opaque original to be copied and the light for exposure of the diazotype material passes through it and is reflected by the surface of the original. The efficiency of the process involving the production of a transition or intermediate print depends upon the opacity of the azo dye image produced upon such intermediate or transition print to ultraviolet light and upon the transparency of the background to such light. It depends also upon the visual density of the image produced on the intermediate or transition print since images of poor visual density, such as light yellows on a white or transparent background,

2

though they may have the desired degree of opacity to ultraviolet light, nevertheless have the disadvantages of rendering difficult the detection of flaws in the intermediate image. With such prints, it is necessary to make a contrast print of good visual density from the intermediate before such flaws can be detected, thereby introducing an additional and unnecessary step.

Prints of a deep color having good visual density can be obtained from diazotypes using azo components common to the art for the production of ordinary diazotypes, such as phloroglucin, 2,3-dihydroxynaphthalene and  $\beta$ -naphthol-3,6-disulfonic acid. However, despite the good visual density of the color reproducing the image, its actinic opacity or photographic density is not sufficient to reproduce the image satisfactorily in subsequent copies. The azo dye component used for the production of transition print images must be such as to produce upon coupling with the diazo compound employed a color which will sufficiently absorb the ultraviolet light incident upon it during exposure to prevent light-decomposition of the diazo compound in the areas to be reproduced from the transition copies. Colors of good visual density do not necessarily have this property. It is well known, for instance, that blues, such as are produced from azo components like phloroglucin, are very poor in their ultraviolet absorption characteristics.

Azo components, such as resorcinol, have heretofore been employed in the production of diazotype prints in order to obtain color images having the necessary light absorption characteristics for transition printing. Resorcinol will reproduce the image on the transition print in a sepia or orange-brown color which has good opacity to ultraviolet light and has sufficient depth of color or visual density to assure detection of printing flaws and the like in the developed intermediate print. Other azo components have been suggested which will produce images of good opacity or covering power when used in combination with polyhydroxy azo components, such as phloroglucinol and resorcinol. These azo components are acetoacetyl derivatives of mono-amines and are disclosed in Patent #1,989,065. However, although these acetoacetyl derivatives of mono-amines may produce satisfactory results as shaders for other colors which may lack the necessary covering power, particularly in copying half-tones or too light lines, they do not produce satisfactory images when used as self colors, that is, when the acetoacetyl derivatives of mono-amines, such as the cyclohexyl acetoacetic acid amide and the like disclosed in Patent #1,989,065, are used as the only azo components for the development of a diazotype print, the

image produced does not have a satisfactory shade or tone value.

It has now been found that certain cyanacetamides containing an active methylene group are especially effective as azo components for diazotype reproduction. These cyanacetamides containing active methylene groups may be represented by the formula



wherein R is a nitrogen containing radical of the group consisting of amino, arylamino, aralkylamino,  $\alpha$  - iminodihydroheterocyclic (such as -quinolyl and -benzthiazole radicals), carbamido, thiocarbamido, carbamidino, cyanimido, and carboalkoxyimido. The azo components of this class can be used satisfactorily either alone in the production of self-shades or in combination with other azo components for shading purposes. In either case, the resulting images will have excellent properties of opacity to ultraviolet light and covering power. When used for shading purposes in combination with such azo components as phloroglucinol, 2,3-dihydroxynaphthalene or 2,3-dihydroxynaphthalene sulfonic acid, excellent neutral blacks having improved opacity to ultraviolet light are obtained. Examples of cyanacetamides having active methylene groups of this class are

1. Cyanacetamide



2. Cyanacetanilide



3. p-Hydroxy cyanacetanilide



4. Cyanacetbenzylamide



5. 1-methyl-2 $\omega$ -cyanacetyliminodihydroquinoline



6. Cyanacetylurea



7. Cyanacetylthiourea



8. Cyanacetylguanidine



9. Cyanacetylcyanamide



10. Cyanacetylthiurethane



11. 1 -  $\omega$  - cyanacetylimino - 2 - methyl-5-ethoxy-dihydrobenzothiazole



In the preparation of diazotype materials intended for use as intermediate or transition print media in accordance with this invention, a suitable transparent base, such as transparentized paper, cellulose acetate film or other transparent material, is coated by means known to the art with a light sensitive composition containing suitable diazo compounds. Where it is desired to make a two-component diazotype layer on the support or base material for development by the dry developing method, the azo component is also incorporated into the coating composition. Where one-component diazotype layers are desired, the azo component is added to an alkaline developing solution and after exposure of the diazotype, the exposed image is developed by contacting with the alkaline developing solution by means known to the art. In the preparation of coating compositions for two-component diazotype layers, the coating solution may also contain such other materials as are ordinarily used in the preparation of diazotype two-component light sensitive coating compositions. These include stabilizing materials, such as citric acid, phosphoric acid and thiourea; swelling agents for cellulose acetate and other cellulosic ester bases, such as isopropanol, and shade intensifying agents, such as nickel sulfate. In the preparation of light sensitive layers on paper for the production of neutral black images or dark tone images which may or may not be intended for reproduction of further copies, it is preferable to employ a two-component coating composition which will contain one or more dark tone producing azo components, preferably such as will produce blue shades with the diazo compounds employed in combination with the nitrile acetyl amide azo components of this invention. The diazo compound or compounds and other adjuvants are added to the coating composition and the paper used as a carrier for the light sensitive layer is coated in the same manner as the transparentized paper or cellulosic film base material in the case of the transition print media. As diazo compounds, any suitable light sensitive diazo compound which will couple with the azo components to reproduce a colored image, may be employed. We prefer, however, to use diazo compounds derived from p-diamines of the benzene series, particularly when two-component coating compositions are employed. As is well known in the art, this class of diazo compounds is especially suitable for the production of two-component diazotype photosensitized papers. Other diazo compounds have been found suitable for use, such as diazo anhydrides of aminohydroxynaphthalene compounds, but are less extensively employed. The p-diamines most generally used for production of the diazo compounds are those wherein one of the amino groups is unsubstituted for diazotization and the other is substituted by such groups as alkyl, alkoxy-alkyl, aryl, aralkyl, alkylol, cycloaliphatic and heterocyclic groups. Examples of these amines from which the diazo compounds are derived include N-hydroxyethyl-N-methylamino-p-aminobenzene; p-amino-diphenylamine; 1-mono-methylamino-2 (or 3) -methyl-4-amino-benzene; 1 - N - hydroxyethyl-N-ethylamino-3-methyl - 4 - aminobenzene; 1-diethylamino-3-ethoxy - 4 - aminobenzene; 4-amino-1-benzoyl-amino-2,5-diethoxybenzene; p-amino-N-diethyl-aniline; 1-N,N-dihydroxyethylamino-3-chloro-4-aminobenzene; p-amino-N-ethyl-N-benzylamine; 1-ethyl-4-aminobenzene; 1-N-hydroxy-

ethyl-N-ethylamino-4-aminobenzene; p-phenylene diamine; 4-amino-N,N-dihydroxyethylamine; p-(4'-ethoxyphenyl)-amino-2,5-diethoxyaniline; 1-N-ethylamino-2-methyl-4-aminobenzene; 1-dimethyl-amino-3-methoxy-4-aminobenzene; N,N-dimethyamino-p-aminobenzene; 1-dimethylamino-3-methyl-4-aminobenzene; p-aminophenyl morpholine and 2-amino-1-naphthol-5-sulfonic acid. The diazo derivatives of these amines are used in the form of their stabilized salts, such as the  $ZnCl_2$ ,  $CdCl_2$  or  $SnCl_2$  double salts, fluoro borates, aryl or alkyl sulfonates, and acid sulfates of the diazonium chloride.

The following specific examples will serve to illustrate further the invention, it being understood, however, that they are not intended to limit its scope. Unless otherwise stated, the parts are by weight.

*Example 1*

Transparentized paper is coated with a coating solution containing the following ingredients per 100 cc. of water containing 5% of alcohol:

4.0 grams cyanacetanilide  
3.8 grams N-methyl-N-hydroxyethyl-p-benzene diazonium chloride- $ZnCl_2$  double salt  
4.0 grams thiourea  
8.0 grams citric acid  
2.0 grams phosphoric acid.  
5.0 grams  $ZnCl_2$

The resulting coated paper or diazotype has good precoupling stability during prolonged storage. After drying the coating in the usual manner, the diazotype is exposed to light under a positive and the image developed with ammonia fumes. The image of the positive original is thus obtained in a light brown colored positive print. The dye or color areas reproducing the image have good fade and wash-fastness properties and excellent opacity to ultra-violet light. The print can be used as a transition print for the reproduction of further diazotype copies or other photo reproductions.

*Example 2*

Transparentized paper is coated with a coating solution containing the following ingredients per 100 cc. of water containing 5% of alcohol:

2.8 grams cyanacetylurea  
3.8 grams N-methyl-N-hydroxyethyl-p-benzene diazonium chloride- $ZnCl_2$  double salt  
4.0 grams thiourea  
8.0 grams citric acid  
2.0 grams phosphoric acid  
5.0 grams zinc chloride

The resulting coated transparency has good precoupling stability during prolonged storage. After drying the coating and exposing to light under a positive and developing the image with ammonia fumes, a reproduction of the positive is obtained in a sepia color. The dye image has good fade and wash-fastness properties and excellent opacity to ultraviolet light. Therefore, it can be used as a transition print in the reproduction of further diazotype copies or other photoprint copies.

*Example 3*

Transparentized paper is coated with a diazotype coating solution containing the following

ingredients per 100 cc. of water containing 5% of alcohol:

3.0 grams cyanacetamide  
3.2 grams 1-(N-ethylamino)-2-methyl-4-benzene diazonium chloride- $ZnCl_2$  double salt  
4.0 grams thiourea  
8.0 grams citric acid  
2.0 grams phosphoric acid  
5.0 grams  $ZnCl_2$

The resulting coated paper or diazotype material has good precoupling stability during prolonged storage. After drying the coating in the usual manner, the diazotype is exposed to light under a pattern, design or picture to be reproduced and the image is developed with ammonia fumes. A positive image of the original is thus obtained in a sepia color. The dye or color areas reproducing the density sections of the original have good fade and wash-fastness properties and show excellent opacity to ultra-violet light. The print, therefore, can be used as a transition or intermediate print for the reproduction of further diazotype copies or other photo-reproductions.

Upon substituting 3.5 grams cyanacetbenzylamide, 3.6 grams 1-(N-ethyl-N-hydroxyethylamino)-3-methyl-4-benzene diazonium chloride- $ZnCl_2$  double salt or 3.3 grams cyanacetylethylurethane and 3.5 grams N-ethyl-N-hydroxyethyl-p-benzene diazonium chloride- $ZnCl_2$  double salt for the coupling component and diazo compound of this example, respectively, diazotype materials having the same properties and reproducing the original in images of the same color as above are obtained.

*Example 4*

A diazotype coating solution containing the following ingredients per 100 cc. of a 5% aqueous solution of alcohol is made up:

1.5 grams cyanacetanilide  
45 3.0 grams 2,3-dihydroxynaphthalene-6-sulfonic acid  
0.15 grams 2,3-dihydroxynaphthalene  
3.2 grams N-ethyl-N-hydroxyethyl benzene-p-diazonium chloride- $ZnCl_2$  double salt  
50 5.0 grams  $ZnCl_2$   
10.0 grams citric acid  
2.0 grams phosphoric acid  
5.0 grams thiourea

Upon using this coating solution to produce a diazotype coating on transparentized diazotype paper stock and upon drying the coating in the usual manner, a diazotype layer having excellent precoupling stability is obtained. Upon exposing the thus sensitized transparentized paper to light under a pattern, design or picture to be reproduced and developing with ammonia fumes, a reproduction of the original in a black shade on a clear background is obtained. This dye image has good fade and wash-fastness properties and excellent opacity to ultraviolet light. Therefore, it can be used as a transition or intermediate print in the reproduction of further diazotype copies or other photoprint copies.

If a non-transparentized diazotype paper stock is used in the coating step and the usual diazotype procedure followed of drying and exposing under a pattern followed by ammonia development, an excellent black reproduction against a white background results.

## Example 5

Transparentized diazotype paper stock is coated with a coating solution containing the following ingredients per 100 cc. of water containing 5% of alcohol:

- 3.2 grams of cyanacetylthiourea
- 3.5 grams N,N-dihydroxyethyl-p-benzene diazonium chloride-CdCl<sub>2</sub> double salt
- 4.0 grams thiourea
- 8.0 grams citric acid
- 2.0 grams phosphoric acid
- 5.0 grams ZnCl<sub>2</sub>

The resulting coated paper or diazotype material has good precoupling stability during prolonged storage. After drying the coating in the usual manner, the diazotype is exposed to light under a pattern or other original to be reproduced and the image is developed with ammonia fumes. The image of the original is thus obtained in a sepia colored positive print. The dye or color areas reproducing the density areas of the original have good fade and wash-fastness properties and excellent capacity to ultraviolet light. The print, therefore, can be used as a transition or intermediate print for the reproduction of further diazotype copies or other photo-reproductions.

Upon substituting for the 3.2 grams cyanacetylthiourea coupling component and the 3.5 grams N,N-dihydroxyethyl-p-benzene diazonium chloride-CdCl<sub>2</sub> double salt diazo compound of this example, the following combinations of coupling components and diazo compounds, diazotype coatings having the same properties as the coatings of this example are obtained:

- (1) 3.3 grams cyanacetylguanidine
- 3.2 grams N-phenylamino-p-benzene diazonium acid sulfate
- (2) 3.1 grams cyanacetylcyanamide
- 3.5 grams 1-(N-ethyl - N - hydroxyethylamino)-3-methyl benzene-p - diazonium chloride-ZnCl<sub>2</sub> double salt
- (3) 3.4 grams cyanacetylethylurethane
- 3.8 grams N,N-diethylamino benzene-p- diazonium chloride-ZnCl<sub>2</sub> double salt
- (4) 3.4 grams 1- $\omega$ -cyanacetyllimino-2-methyl-5-ethoxydihydrobenzothiazole
- 3.5 grams 1-(N-ethyl - N - hydroxyethyl) amino-3-methyl benzene - p - diazonium chloride-ZnCl<sub>2</sub> double salt
- (In this case the coating solution contains 10% alcohol per 100 cc. of water)
- (5) 3.2 grams 1-methyl-2- $\omega$ -cyanacetyllimino dihydroquinoline
- 3.5 grams N-hydroxyethyl-N-methyl benzene-p-diazonium chloride-ZnCl<sub>2</sub> double salt
- (In this case the coating solution contains 10% alcohol per 100 cc. of water)

We claim:

1. A diazotype photoprinting material comprising a light sensitive diazonium salt of a p-diamine

of the benzene series and an azo component selected from the class consisting of cyanacetylamides of the following formula



wherein R is a nitrogen containing radical of the class consisting of amino, arylamino, aralkylamino,  $\alpha$ -iminodihydroheterocyclic, carbamido, thiocarbamido, carbamidino, cyanimido, and carboalkoxylimido radicals.

2. A diazotype photoprinting material comprising a light sensitive diazonium salt of a p-diamine of the benzene series and as an azo component cyanacetanilide having the structural formula



3. A diazotype photoprinting material comprising a light sensitive diazonium salt of a p-diamine of the benzene series and as an azo component cyanacetylurea having the structural formula



4. A diazotype photoprinting material comprising a light sensitive diazonium salt of a p-diamine of the benzene series and as an azo component cyanacetbenzylamide having the structural formula



5. A diazotype photoprinting material comprising a light sensitive diazonium salt of a p-diamine of the benzene series and as an azo component cyanacetamide having the structural formula



6. A diazotype photoprinting material comprising a light sensitive diazonium salt of a p-diamine of the benzene series and as an azo component cyanacetylthiourea having the structural formula



WILLIAM H. VON GLAHN.  
LESTER N. STANLEY.

## REFERENCES CITED

50 The following references are of record in the file of this patent:

## UNITED STATES PATENTS

| Number    | Name           | Date          |
|-----------|----------------|---------------|
| 1,989,065 | Schmidt et al. | Jan. 22, 1935 |
| 2,108,602 | Mannes et al.  | Feb. 15, 1938 |
| 2,217,189 | Sus            | Oct. 8, 1940  |
| 2,312,040 | Kendall et al. | Feb. 23, 1943 |
| 2,436,007 | Kendall et al. | Feb. 17, 1948 |
| 2,453,661 | Glass          | Nov. 9, 1948  |